



US005885124A

# United States Patent [19]

Hattori

[11] Patent Number: 5,885,124

[45] Date of Patent: Mar. 23, 1999

[54] **FABRICATION OF FIELD EMISSION ELEMENT WITH SMALL APEX ANGLE OF Emitter**5,720,641 2/1998 Hattori ..... 445/24  
5,720,642 2/1998 Hattori ..... 445/24  
5,749,762 5/1998 Nakamoto et al. ..... 445/50[75] Inventor: **Atsuo Hattori**, Hamamatsu, JapanPrimary Examiner—Kenneth J. Ramsey  
Attorney, Agent, or Firm—Ostrolenk, Faber, Gerb & Soffen,  
LLP[73] Assignee: **Yamaha Corporation**, Japan[21] Appl. No.: **778,454****ABSTRACT**[22] Filed: **Jan. 3, 1997**

A method of fabricating a field emission element includes the steps of: forming an overhang portion in a substrate, the overhang portion including two opposing parts in cross section; depositing a sacrificial film on the overhang portion with two opposing parts, the sacrificial film including two opposing parts in cross section; chemically reacting the sacrificial film with two opposing parts to expand the volume of the sacrificial film and make the two opposing parts partially contact each other; depositing a field emission cathode film on the sacrificial film with contacted two opposing parts; and removing part of, or the whole of, the sacrificial film to expose a tip of the field emission cathode film.

[30] **Foreign Application Priority Data**

Jan. 8, 1996 [JP] Japan ..... 8-001039

[51] **Int. Cl.<sup>6</sup>** ..... **H01J 9/02**[52] **U.S. Cl.** ..... **445/24; 445/50**[58] **Field of Search** ..... **445/24, 50**[56] **References Cited**

## U.S. PATENT DOCUMENTS

5,141,459 8/1992 Zimmerman ..... 445/24

5,203,731 4/1993 Zimmerman ..... 445/24

5,334,908 8/1994 Zimmerman ..... 313/336

**16 Claims, 19 Drawing Sheets**

**FIG.1A****FIG.1B****FIG.1C**

**FIG. 1D****FIG. 1E****FIG. 1F**

***FIG. 1G***



**FIG. 2A****FIG. 2B****FIG. 2C**

**FIG.3**

**FIG.4A****FIG.4B****FIG.4C**

**FIG.4D****FIG.4E**

**FIG.5A****FIG.5B****FIG.5C**

***FIG. 6***

**FIG.7A****FIG.7B**

***FIG.8***

**FIG.9A****FIG.9B****FIG.9C**

**FIG. 10A****FIG. 10B****FIG. 10C**

**FIG.11**

**FIG.12A****FIG.12B**

FIG. 13



FIG. 14



**FIG. 15**

**FIG. 16A**  
**PRIOR ART**



**FIG. 16B**  
**PRIOR ART**



## FABRICATION OF FIELD EMISSION ELEMENT WITH SMALL APEX ANGLE OF Emitter

### BACKGROUND OF THE INVENTION

#### a) Field of the Invention

The present invention relates to a manufacture method of a field emission element.

#### b) Description of the Related Art

A field emission element emits electrons from a sharp tip of an emitter by utilizing electric field concentration. For example, a flat panel display can be structured by using a field emitter array (FEA) having a number of emitters disposed on the array. Each emitter controls one pixel of the display.

FIGS. 16A and 16B illustrate conventional manufacture methods of a field emission element.

As shown in FIG. 16A, on a substrate 101 having a recess with a vertical side, a sacrificial film 103 is deposited by a deposition method having poor step coverage. The upper surface of the sacrificial film 103 has a tapered portion at the recess. An emitter electrode (cathode) 105 formed by using this sacrificial film 103 as a mold has a tip A. If the radius of curvature of the tip A of the emitter electrode 105 is large, an electric field is hard to concentrate and the electrical performance is not good.

As shown in FIG. 16B, if a sacrificial film 103 is deposited thick on a substrate 101 having a recess, two side wall parts in cross section of the sacrificial film 103 at the recess become partially in unison so that an emitter electrode 105 having a relatively small apex angle of the emitter tip can be formed.

With this method, it is necessary to deposit the sacrificial film thick so that the tip of the emitter electrode is formed at an upper position remote from the substrate 101. If a field emission element has a gate electrode in addition to an emitter electrode, this gate electrode is generally formed near at the boundary between the substrate 101 and the sacrificial film 103, although not shown in FIG. 16B. With the method illustrated in FIG. 16B, the emitter electrode 105 is formed remotely from the gate electrode so that a high drive voltage of the field emission element is required and the electrical performance is lowered.

A large radius of curvature of the emitter electrode tip makes an electric field hard to concentrate, lowering the performance of the field emission element. A relative position of the emitter and gate electrodes greatly influences the performance of the field emission element.

### SUMMARY OF THE INVENTION

It is an object of the present invention to provide a manufacture method of a field emission element having a field emission cathode (emitter) with a small apex angle and radius of curvature of the emitter tip.

It is another object of the present invention to provide a manufacture method of a field emission element having a field emission cathode, capable of positioning an emitter tip with high precision.

According to one aspect of the present invention, there is provided a method of fabricating a field emission element comprising: a step of forming an overhang portion in a substrate, the overhang portion including two opposing parts in cross section; a sacrificial film depositing step of depositing a sacrificial film on the overhang portion with two

opposing parts, the sacrificial film including two opposing parts in cross section; a reacting step of chemically reacting the sacrificial film with two opposing parts to expand the volume of the sacrificial film and make the two opposing parts partially contact each other; a depositing step of depositing a field emission cathode film on the sacrificial film with contacted two opposing parts; and an electrode exposing step of removing part of, or the whole of, the sacrificial film to expose a tip of the field emission cathode film.

The two opposing parts of the sacrificial film are made partially in contact with each other by chemical reaction. A sharp valley is formed at this contact area, the sharp valley having a cross section like two contacted circles. By using this valley as a mold, a field emission emitter having a small apex angle and radius of curvature of the emitter tip can be manufactured.

According to another aspect of the present invention, there is provided a method of fabricating a two-electrode field emission element wherein the reaction step of the first mentioned method is a step of chemically reacting only part of the sacrificial film to use the other part not chemically reacted as a gate electrode made of semiconductor or conductive material, the field emission cathode film is an emitter electrode made of conductive material, and the electrode exposing step is a step of exposing the tip of the emitter electrode and the head of the gate electrode.

The relative position of the emitter and gate electrode can be set precisely by properly selecting the process conditions of the step of depositing the sacrificial film on the overhang portion with opposing two parts and the step of chemically reacting the sacrificial film.

### BRIEF DESCRIPTION OF THE DRAWINGS

FIGS. 1A to 1G are diagrams illustrating the manufacture steps of a field emission element according to an embodiment of the invention.

FIGS. 2A to 2C are diagrams illustrating three methods of reinforcing an emitter electrode with a support substrate.

FIG. 3 is a diagram illustrating another method of forming a first sacrificial film.

FIGS. 4A to 4E are diagrams illustrating the manufacture steps of a field emission element according to another embodiment of the invention.

FIGS. 5A to 5C are diagrams illustrating the manufacture steps of a field emission element according to still another embodiment of the invention.

FIG. 6 is a diagram illustrating the manufacture steps of a two-electrode field emission element according to an embodiment of the invention.

FIG. 7A is a schematic diagram showing a relative position of emitter and gate electrodes, and FIG. 7B is a graph showing a relationship between a distance between emitter and gate electrodes and a maximum field intensity.

FIG. 8 is a diagram illustrating the manufacture steps of a two-electrode field emission element according to another embodiment of the invention.

FIGS. 9A to 9C are diagrams illustrating three methods of reinforcing a two-electrode field emission element with a support substrate.

FIGS. 10A to 10C are diagrams illustrating the manufacture steps of a three-electrode field emission element according to an embodiment of the invention.

FIG. 11 is a perspective view of a three-electrode field emission element according to an embodiment of the invention.

FIGS. 12A and 12B are diagrams showing the three-electrode field emission element shown in FIG. 11 turned upside down. FIG. 12A shows an emitter electrode having a needle-like tip, and FIG. 12B is a perspective view of an emitter electrode having a wedge-like tip extending in one direction.

FIG. 13 is a cross sectional view of a flat panel display using field emission elements.

FIG. 14 is a perspective view partially in section of a flat panel display using field emission elements.

FIG. 15 is a circuit diagram of a flat panel display.

FIGS. 16A and 16B are cross sectional views of conventional field emission elements.

#### DETAILED DESCRIPTION OF THE PREFERRED EMBODIMENTS

FIGS. 1A to 1G are diagrams illustrating the manufacture steps of a field emission element according to an embodiment of the invention. In the following, the manufacture steps of an emitter (cathode) constituting a field emission element will be described.

As shown in FIG. 1A, a substrate 10 is structured by a starting substrate 10a and a lamination film 10b of about 140 nm thick stacked upon the starting substrate 10a. For example, the starting substrate 10a is made of Si, and the lamination film 10b is made of SiN<sub>x</sub>.

The lamination film 10b may be made of SiO<sub>2</sub> instead of SiN<sub>x</sub>. The starting substrate 10a may be made of Al. If Al is used, the lamination film 10b is made of AlN<sub>x</sub>, Al<sub>2</sub>O<sub>3</sub>, or the like. In the following, it is assumed that the starting substrate 10a is made of Si and the lamination film 10b is made of SiN<sub>x</sub>.

A resist film having a predetermined pattern is formed on the lamination film 10b. By using the resist pattern as a mask, the lamination film 10b is selectively etched to form a hole 12 shown in FIG. 1B in the lamination film 10b so that a surface of the starting substrate 10a is exposed from an aperture of the hole 12. A lamination film 10c having two opposing parts in cross section is therefore formed. The hole 12 is circular as viewed down from the upper position and corresponds to a gate hole. The lamination film 10c is formed so as to surround the circular hole 12 as viewed down from the upper position. This selective etching is performed by reactive ion etching (RIE) using SF<sub>6</sub> containing etching gas. The hole 12 has a diameter of about 0.5 μm and a depth of about 140 nm.

By using the lamination film 10c as an etching mask, the starting substrate 10a is wet etched to form a hole 12a in the starting substrate. A substrate 10d is therefore formed. The hole 12a forms a hollow space and has a diameter of about 1.5 μm and a depth of about 0.5 μm. Isotropical wet etching is performed through the hole 12 to etch the starting substrate 10a not only along the vertical direction of the substrate 10a but also along the horizontal direction in the cross-section of the starting substrate 10a. Therefore, the starting substrate 10a is etched partially at the underneath of the lamination film 10c. The lamination film 10c extends like a hood near the hole 12a. As shown in FIG. 1C, an overhang portion 13 is therefore formed having two opposing parts in cross section separated along the horizontal direction of the substrate. The two opposing parts in section is called hereinafter simply "two parts".

As shown in FIG. 11D, a first sacrificial film 15a made of, for example, polysilicon is deposited by CVD about 0.3 μm thick on the lamination film 10c with two parts. This CVD

is performed under the conditions of a temperature of 625° C., a pressure of 30 Pa, and a supply of SiH<sub>4</sub> diluted with He at 0.6 slm. At the same time, a first sacrificial film 15b is also deposited through an opening on the substrate 10d at the bottom of the hole 12a. The first sacrificial film 15a also has two parts separated by a distance of about 0.1 μm.

The first sacrificial films 15a and 15b may be made of amorphous silicon, WSi<sub>x</sub>, MoSi<sub>x</sub>, TaSi<sub>x</sub>, Al, Ta, Mo, or Ti, instead of polysilicon. Sputtering may be used instead of CVD. For example, the first sacrificial films 15a and 15b of amorphous silicon may be formed by a DC sputtering system using, as a target, polysilicon which contains P or B. For example, sputtering is performed under the conditions of a power of 1 kW and an Ar gas pressure of 8 mTorr.

Next, as shown in FIG. 1E, the surfaces of the first sacrificial films 15a and 15b are oxidized by wet oxidation to form reacted films 16c and 16d made of, for example, SiO<sub>2</sub>. The volume of the first sacrificial film 15a with two parts expands by about 0.1 μm by the oxidation and the two parts contact each other to form a continuous film of a reacted film 16c having only one part. The first sacrificial film 15a shown in FIG. 1D not oxidized forms a first sacrificial film 15c. In order to fill the space of 0.1 μm, the surface of the first sacrificial film 15a with two parts is expanded by 0.05 μm per one part. To obtain the surface volume expansion of 0.05 μm, polysilicon is oxidized by about 0.05 μm thick.

For example, wet oxidation is performed by using a vertical furnace under the conditions of a furnace temperature of 850° C., a supply of H<sub>2</sub> gas at 30000 cc/min, and a supply of O<sub>2</sub> gas at 20000 cc/min.

If the chemical reaction is stopped immediately after the two parts in cross section of the first sacrificial film contact each other by the volume expansion, a valley having an acute angle can be formed at the contact area. This contact area has an acute angle area having a cross section like two contacted circles or ellipses. If oxidation continues after the opening is closed, the contact point of the two parts of the sacrificial film gradually moves up. Even with this change, the apex angle at the contact area maintains an acute angle. By using this acute angle area as a mold, an emitter electrode is formed.

As shown in FIG. 1F, an emitter electrode 17 made of, for example, TiN is deposited on the reacted film 16c about 0.2 μm by reactive sputtering. For example, the reactive sputtering is performed by using a DC sputtering system under the conditions of a power of 5 kW, a pressure of 4 mTorr, a target of Ti, a supply of N<sub>2</sub> gas at 84 sccm, and a supply of Ar gas at 56 sccm. The emitter electrode 17 may be made of Mo, Cr, Ti, or W, instead of TiN.

The substrate 10d is wet etched by HF+HNO<sub>3</sub>+H<sub>2</sub>O, and thereafter tsm reacted film 16c is wet etched by HF+NH<sub>4</sub>F to expose the tip of the emitter electrode as shown in FIG. 1G.

It can be predicted that the tip of the emitter electrode 17 has a projection of 0.3 to 0.8 μm high, an apex angle of about 20° and a radius of curvature of about 10 nm. With the manufacture method described above, the radius of curvature and apex angle or the tip of the emitter electrode 17 can be made small so that an electric field concentrates easily at the tip of the emitter electrode.

FIGS. 2A to 2C are diagrams illustrating three methods of reinforcing an emitter electrode 17 with a support substrate 18. Since the emitter electrode 17 is as thin as about 0.2 μm, it is desired to reinforce the emitter electrode 17 with the support substrate 18.

FIG. 2A illustrates the first method. A bottom recess of the emitter electrode manufactured as shown in FIG. 1F is filled with a planarizing film 19a of, for example, an SOG film. Thereafter, the planarizing film 19a is abraded by chemical mechanical polishing (CMP) or by etch-back to planarize the bottom surface of the emitter electrode 17. The planarizing film 19a may be formed by reflowing PSG or BPSG instead of using the SOG film.

Next, a support substrate 18 is adhered to the emitter electrode 17. The support substrate 18 is made of, for example, glass, quartz, or  $\text{Al}_2\text{O}_3$ . Thereafter, the process illustrated in FIG. 1G is performed.

FIG. 2B illustrates the second method. Adhesive 19b such as low melting point glass is reflowed on the emitter electrode in the state shown in FIG. 1F to adhere the emitter electrode 17 and a support substrate 18 together. Thereafter, the process illustrated in FIG. 1G is performed. The adhesive 19b also serves to planarize the bottom surface of the emitter electrode 17.

In place of the low melting point glass, Al may be used as the adhesive 19b. In this case, the emitter electrode 17 and support substrate 18 may be adhered by anodic bonding using electrostatic forces generated upon application of a high voltage of 1 kV and maintaining the temperature at 400° to 500° C. If Al is used as the adhesive 19b, the adhesive 19b may be used as an emitter wiring.

FIG. 2C illustrates the third method. The bottom recess of the emitter electrode in the state shown in FIG. 1F is filled with a planarizing film 19a made of, for example, W. Thereafter, the planarizing film 19a is etched back to planarize the bottom surface of the emitter electrode 17. A support substrate 18 is adhered to the emitter electrode 17 by using adhesive 19b such as Al. Thereafter, the process illustrated in FIG. 1G is performed.

In this embodiment, the process of forming the first sacrificial film 15a shown in FIG. 1D is important for determining the shape of the emitter electrode. For example, the distance between two parts of the first sacrificial film 15a is preferably about 0.1  $\mu\text{m}$ . This distance between the two parts of the first sacrificial film 15a may be adjusted by another method described in the following.

FIG. 3 is a diagram illustrating a method of forming the first sacrificial film. After the process illustrated in FIG. 1G, first sacrificial films 15d and 15e are deposited thick by CVD or the like. The first sacrificial film 15d is controlled to have two parts. Thereafter, the thickness of the first sacrificial film 15a is adjusted to the thickness shown in FIG. 1D, by isotropic wet etching. This wet etching is performed by using, for example,  $\text{HG}+\text{HNO}_3+\text{H}_2\text{O}$ . The bottom surface of the overhang portion of the first sacrificial film 15d may be made thin. Thereafter, the processes starting from FIG. 1E are executed.

In the process illustrated in FIG. 1E, the reacted films 16c and 16d are formed by wet oxidation. Instead of wet oxidation, these reacted films may be formed by nitridation, anodic oxidation, silicide reaction, ion implantation, or the like. In the following, each of these methods will be described.

With nitridation, the reacted film 16c of  $\text{SiN}_x$  can be formed from the first sacrificial film 15a of polysilicon. For example, nitridation is performed under the conditions of a temperature of 1050° C., an RF power of 10 kW, a pressure of 130 Pa, and a supply of  $\text{NH}_3$  at 1 slm.

In order to oxidize the first sacrificial film 15a of Al through anodic oxidation, borate or phosphate may be used as electrolytic solution, and a voltage of 10 to 80 V is applied between the anode Al and a carbon cathode.

Next, the methods of forming a reacted film through silicide reaction and ion implantation will be described with reference to FIGS. 4A to 4E and FIGS. 5A to 5C.

FIGS. 4A to 4E illustrate the method of manufacturing a field emission element by using silicide reaction.

The process illustrated in FIG. 4A follows the process illustrated in FIG. 1D. On the first sacrificial film 15a made of, for example, polysilicon or amorphous silicon, a second sacrificial film 21a made of, for example, Ti is formed. Instead of Ti, the second sacrificial film 21a may be made of refractory metal such as Ta, Mo, and W. In this specification, refractory metal includes Ti, Ta, Mo, and W.

Next, as shown in FIG. 4B, as the substrate is heated to 400° to 600° C., silicide reaction proceeds and a reacted film 22 of TiSi is formed between the first sacrificial film 15c of Si and the second sacrificial film 21b of Ti.

The second sacrificial film 21b is etched by sulfuric acid to expose the surface of the reacted film 22 as shown in FIG. 4C. By using the valley formed on the surface of the reacted film 22 as a mold, an emitter electrode is formed.

As shown in FIG. 4D, an emitter electrode 17 made of, for example, TiN is formed on the reacted film 22. The reacted film 22 made of TiSi is etched by hydrofluoric acid to expose the tip of the emitter electrode 17 as shown in FIG. 4E.

FIGS. 5A to 5C illustrate the method of manufacturing a field emission element by using ion implantation.

The process illustrated in FIG. 5A follows the process illustrated in FIG. 1D. Into the first sacrificial film 15a made of, for example, polysilicon or amorphous silicon, oxygen ions are implanted under the conditions of a dose of  $1 \times 10^{18} \text{ cm}^{-2}$  and an acceleration energy of 20 to 40 keV to form an ion implanted layer 25 in the surface area of the first sacrificial film 15a. Instead of oxygen, nitrogen ions may be implanted.

Next, as shown in FIG. 5B, the substrate is annealed to grow oxide films 16c and 16d in an oxygen ambient. A first sacrificial film 15c corresponds to a portion of the first sacrificial film 15a shown in FIG. 5A not oxidized.

In the oxygen ion implanted layer 25, an oxide film grows fast. As the oxide film 16c grows, the two parts of the first sacrificial film 15a contact each other. By using a valley formed at the contact area as a mold, an emitter electrode is formed.

As shown in FIG. 5C, an emitter electrode 17 made of, for example, TiN is formed on the oxide film 16c. Thereafter, the oxide film 16c is wet etched by  $\text{HF}+\text{NH}_4\text{F}$  to expose the tip of the emitter electrode 17 in such a manner as illustrated in FIGS. 1G and 4F.

In the description with reference to FIGS. 5A, B impurity ions (reaction species) such as oxygen and nitrogen are implanted into the surface area of the first sacrificial film 15a. Ions may be implanted into the intermediate area in depth of the first sacrificial film 15a and the impurity concentration of the surface area may be made low, by changing the ion implantation conditions.

As will be described later, the first sacrificial film 15c shown in FIG. 5C is used as the gate electrode of a two-electrode or three-electrode element. If ions are implanted into the surface area of the first sacrificial film 15a shown in FIG. 5A, the tip of the emitter electrode 17 is formed at a relatively high position, and the distance (gate diameter) between the two parts of the gate electrode 15c becomes short.

If ions are implanted into the relatively deep area of the first sacrificial film 15a, the tip of the emitter electrode 17 is

formed at a relatively low position, and the distance (gate diameter) between the two parts of the gate electrode 15c becomes long.

The emitter electrode manufacture methods have been described so far. Next, a method of manufacturing another type of a field emission element of a two-electrode element will be described.

FIG. 6 is a diagram illustrate the method of manufacturing a two-electrode element (so-called a diode). First, an element shown in FIG. 1F is formed by the above described processes. Thereafter, the substrate 10d, reacted film 16d, and part of the reacted film 16c are etched. By partially removing the reacted film 16c and leaving the reacted film 16e unetched as shown in FIG. 6, the tip of the emitter electrode 17 is exposed. The substrate 10d is etched, for example, by  $\text{HF}+\text{HNO}_3+\text{H}_2\text{O}$ , and the reacted films are etched, for example, by  $\text{HF}+\text{NH}_4\text{F}$ .

If the first sacrificial film is made of conductive polysilicon or amorphous silicon, the first sacrificial film 15c, which is unreacted, can be used as a gate electrode. The two-electrode element has two electrodes—the emitter electrode 17 and gate electrode 15c. The reacted film 16e electrically isolates the emitter electrode 17 and gate electrode 15c. The lamination film 10c may be removed by etching.

A relative position of the emitter electrode 17 and gate electrode 15c plays an important role of a two-electrode element. A shorter distance between the emitter electrode 17 and gate electrode 15c is principally better. It is therefore desired to position the tip of the emitter electrode 17 near at a straight line interconnecting the two parts of the gate electrodes 15c.

FIG. 7A is a schematic diagram showing the relative position of the gate electrode 15c and emitter electrode 17. The relative position is turned upside down from that shown in FIG. 6. A distance Zge is a distance from the tip of the emitter electrode 17 to the center of a thickness td of the gate electrode 15c, along an electron emission direction.

FIG. 7B is a graph showing a relationship between the distance Zge and a maximum field intensity  $E_{\text{max}}$  at the tip of the emitter electrode, with the thickness td of the gate electrode 15c being fixed to  $0.4 \mu\text{m}$ . The abscissa represents the distance Zge, and the ordinate represents the maximum field intensity  $E_{\text{max}}$ .

This graph shows a change in the maximum field intensity  $E_{\text{max}}$  of the emitter electrode as the distance Zge between the emitter and gate electrodes is changed from  $-0.35 \mu\text{m}$  to  $0.25 \mu\text{m}$ . The larger the maximum field intensity  $E_{\text{max}}$ , the more the electric field concentrates on the tip of the emitter electrode and the more the performance of the field emission element is improved. At the distance Zge of  $-0.1 \mu\text{m}$ , the maximum field intensity  $E_{\text{max}}$  takes an extreme value of  $1.16 \times 10^7 \text{ V/cm}$ . Namely, the optimum position of the tip of the emitter electrode 17 is slightly higher in FIG. 7A (slightly lower in FIG. 6) than the center of the thickness of the gate electrode.

The two-electrode element uses the emitter electrode 17 as a cathode and the gage electrode 15c as a control electrode. If the tip of the emitter electrode 17 is set to a proper position, electrons can be easily emitted from the tip of the emitter electrode 17 even at a low control voltage applied to the gate electrode.

The two-electrode element has the emitter electrode 17 with a small apex angle and radius of curvature of the tip so that the performance of the field emission element can be improved.

FIG. 8 shows another example of a two-electrode element. In this two electrode element, the thicknesses of the

gate electrode (first sacrificial film) 15c and the insulating film (reacted film) 16e are different from those of the two-electrode element shown in FIG. 6. The thicknesses of the gate electrode 15c and insulating film 15e can be controlled by changing the thickness of the first sacrificial film deposited on the lamination film 10c and by changing a reaction time or method of the first sacrificial film.

The two-electrode element shown in FIG. 8 has the gate electrode (first sacrificial film) 15c thicker than that of the two-electrode element shown in FIG. 6 and has a smaller diameter of the gate hole than that of the element shown in FIG. 6. In order to increase the thickness of the gate electrode (first sacrificial film) 15c, the first sacrificial film 15a shown in FIG. 1D is deposited more anisotropically.

Anisotropic deposition of the first sacrificial film 15a reduces the diameter of the gate hole. Therefore, even at a low gate-emitter voltage, electrons can be emitted from the emitter electrode. Similar advantages are also obtained by a three-electrode element to be described later.

The first sacrificial film 15a shown in FIG. 1D is anisotropically deposited on the lamination film 10c. This film 15a may be deposited isotropically. However, anisotropic deposition makes the diameter of the hole (gate hole) of the gate electrode smaller and can improve the electrical characteristics.

If the first sacrificial film is isotropically deposited at the process of FIG. 1D, the first sacrificial film 15a deposited at the overhang portion is likely to be integrated with the first sacrificial film 15b deposited on the substrate 10d. It is therefore difficult to form the first sacrificial film 15a having two parts.

According to this embodiment, after the first sacrificial film is formed, it is subjected to chemical reaction to expand its volume so that the position of the tip of the emitter electrode 17 can be controlled precisely.

A film formed by CVD becomes thick approximately proportional to time. In contrast, a film formed by chemical reaction such as oxidation becomes thick approximately proportional to a square root of time. In other words, the film thickness tends to saturate as the time lapses. With oxidation or the like, the film thickness can be controlled more finely and the tip position of the emitter electrode can be controlled more precisely, the more the time lapses. Furthermore, a film having a better uniform quality can be formed by oxidation than CVD.

FIGS. 9A to 9C are diagrams illustrating three methods of reinforcing a two-electrode element with a support substrate 18, similar to the methods described with FIGS. 2A to 2C.

FIG. 9A illustrates the first method. A bottom recess of the emitter electrode 17 is filled with a planarizing film 19a of, for example, an SOG film, a PSG film, or a BPSG film. Thereafter, the planarizing film 19a is etched back by CMP to planarize the bottom surface of the emitter electrode 17. Next, a support substrate 18 is adhered to the emitter electrode 17. The support substrate 18 is made of, for example, glass, quartz, or  $\text{Al}_2\text{O}_3$ .

FIG. 9B illustrates the second method. Adhesive 19b such as low melting point glass is reflowed on the emitter electrode 17 to planarize the bottom surface of the emitter and adhere the emitter electrode 17 and a support substrate 18 together. Al may be used as the adhesive 19b to anodically bond the emitter electrode 17 and support substrate 18.

FIG. 9C illustrates the third method. The bottom recess of the emitter electrode is filled with a planarizing film 19a made of, for example, W. Thereafter, the planarizing film 19a is etched back to planarize the bottom surface of the

emitter electrode 17. A support substrate 18 is adhered to the emitter electrode 17 by using adhesive 19b such as Al.

The manufacture method of a two-electrode element has been described. Next, a manufacture method of another type of a field emission element of a three-electrode element will be described.

FIGS. 10A to 10C are diagrams illustrating a method of manufacturing a three-electrode element (so-called a triode).

First, the element shown in FIG. 1F is manufactured by the previously described processes. Thereafter, a resist film having a predetermined pattern (not shown) is formed on the emitter electrode 17. By using this resist pattern as a mask, slit openings 20 are formed on both sides of an emitter electrode 17a by RIE using Cl<sub>2</sub> containing etchant. An emitter electrode 17b is formed at the outer sides of the slit openings 20.

The diameter of the emitter electrode 17a is about 0.3  $\mu$ m, and the depth of the slit openings is about 0.2  $\mu$ m.

Next, part of the reacted film 16c and the whole of the reacted film 16d are wet etched. For example, HF+NH<sub>4</sub>F is used for wet etching the reacted films 16c and 16d made of SiO<sub>2</sub>.

Part of the reacted film 16c is etched and a reacted film 16f is left unetched as shown in FIG. 10B so that the emitter electrode 17a, gate electrode 15c, and anode electrode 10d are exposed.

FIG. 11 is a perspective view of a three-electrode element. The emitter electrode 17a is integrally formed with the emitter electrode 17b. The gate electrode 15c has a circular hole (gate hole) near at the tip of the emitter electrode 17a. The tip of the emitter electrode 17a has a needle-like sharp edge near at the gate hole of the gate electrode 15c.

FIG. 12 is a perspective view showing the three-electrode element shown in FIG. 11 turned upside down, the emitter electrode 17a being viewed through the substrate via the gate hole of the gate electrode. The tip of the emitter electrode 17a has a needle-like sharp edge. The tip of the emitter electrode 17a may be have different shapes.

FIG. 12B is a perspective view showing a three-electrode element having a slit gate hole of the gate electrode 15c. The emitter electrode 17a has a wedge-like tip extending along the longitudinal direction of the gate hole.

The three-electrode element shown in FIG. 11 has the emitter electrode 17 as a cathode and an anode electrode 10d wherein a positive potential is applied to the gate electrode 15c to emit electrons from the emitter electrode 17a toward the anode electrode 10d.

Also in the case of a three-electrode element, the apex angle and radius of curvature of the tip of the emitter electrode 17a can be made small. The relative position of the emitter electrode 17a and gate electrode 15c can be controlled precisely.

In the above description, the lamination film 10c is made of insulating material such as SiN<sub>x</sub>. Next, forming the lamination film 10c by conductive material will be described.

FIG. 10C is a cross sectional view showing another example of a three-electrode element. A lamination film (first gate electrode) 15f is made of conductive material such as WSi<sub>x</sub>, TaSi<sub>x</sub>, and MoSi<sub>x</sub>. Between the anode electrode 10d and lamination film 15f, an insulating film 10f made of SiO<sub>2</sub>, SiN<sub>x</sub>, or the like is formed. The manufacture method of this three-electrode element will be described next.

The substrate 10 shown in FIG. 1A is constituted of the starting substrate 10a and the lamination film 10b of insu-

lating material stacked on the starting substrate 10a. In the case of the three-electrode element shown in FIG. 10C, on a substrate 10d made of, for example, Si, an insulating film 10f made of SiO<sub>2</sub> or the like and a lamination film 15f made of conductive material are sequentially laminated. Thereafter, the processes described previously are performed to manufacture the three-electrode element shown in FIG. 10C.

By using the conductive lamination film 15f, a lamination of the first gate electrode 15f and second gate electrode 15c forms a low resistance gate electrode. The gate electrodes 15f and 15c are electrically isolated from the anode electrode 10d by the insulating film 10f.

FIG. 13 is a cross sectional view of a flat panel display using field emission elements.

Each field emission element used is an emitter electrode or a two-electrode element formed by the embodiment manufacture method. On a support substrate 41 made of insulating material, a wiring layer 42 made of Al, Cu, or the like and a resistor layer 43 made of polysilicon or the like are formed. On the resistor layer 43, a number of emitter electrodes having a small apex angle and radius of curvature of the emitter tip are disposed to form a field emitter array (FEA). Each gate electrode 45 has an opening (gate hole) near at the tip of each emitter electrode 44 and a voltage can be applied independently to each gate electrode. A plurality of emitter electrodes can also be independently applied with a voltage.

Facing an electron source including the emitter electrode 44 and gate electrode 45, an opposing substrate is disposed including a transparent substrate 46 made of glass, quartz, or the like. The opposing substrate has a transparent electrode (anode electrode) 47 made of ITO or the like disposed under the transparent electrode 46 and a fluorescent member 48 disposed under the transparent electrode 47.

The electron source and opposing substrate are joined together via a spacer 50 made of a glass substrate and coated with adhesive, with the distance between the transparent electrode 47 and emitter electrode 44 being maintained about 0.1 to 5 mm. The adhesive may be low melting point glass.

Instead of the spacer 50 of a glass substrate, a spacer 50 made of adhesive such as epoxy resin with glass beads being dispersed therein may be used.

A getter member 51 is made of Ti, Al, Mg, or the like and prevents emitted gas from attaching again to the surface of the emitter electrode 44.

An air exhaust pipe 49 is coupled to the opposing substrate. By using this air exhaust pipe 49, the inside of the flat display panel is evacuated to about 10<sup>-5</sup> to 10<sup>-9</sup> Torr, and then the air exhaust pipe 49 is sealed by using a burner or the like. Thereafter, the anode electrode (transparent electrode) 47, emitter electrode 44, gate electrode 45 are wired to complete the flat panel display.

FIG. 14 is a perspective view of a flat panel display. A gate electrode 45 has a number of gate holes 53. An emitter electrode 44 is formed in one-to-one correspondence with each gate hole 53. Each emitter electrode is partitioned by an insulating film 54. Electrons emitted from the emitter electrode 44 pass through a vacuum hollow space 52 and collide with a fluorescent member 48 to radiate light therefrom.

The flat panel display is constituted of a plurality of pixels. Each pixel is constituted of a region PQRS made of four emitter electrodes 44 and a corresponding region P'Q'R'S' of the opposing substrate.

## 11

A resistor Layer 43 and a wiring layer 42 formed under the emitter electrodes 44 are partitioned by a planarizing film (insulating film) 55 in unit of pixel (four emitter electrodes).

FIG. 15 is an equivalent circuit diagram of a flat panel display which is made of a field emitter array (FEA) having a number of triodes.

A number of triodes are disposed at cross points between two-dimensionally patterned emitter wirings EW and gate wirings GW. The anode wiring AW of an anode electrode (transparent substrate) 47 of each triode is always maintained at a positive potential. The triodes are two-dimensionally disposed by the emitter wirings EW and gate wirings GW, and the triode at the cross point of the voltage-applied emitter wiring EW and gate wiring GW is selected. 15

The emitter electrode and gate electrode of the selected triode are applied with negative and positive potentials, respectively, so that electrons are emitted from the emitter electrode to the anode electrode.

In the above embodiments, the volume of the first sacrificial film having two parts is expanded by chemical reaction to make the two parts contact with each other and form an acute angle valley at the contact area. By using this valley as a mold, an emitter electrode having a small apex angle and radius of curvature of the emitter tip can be formed. 20

The relative position of the emitter electrode and gate electrode can be determined precisely.

The distance (gate diameter) of the two parts of the gate electrode can be shortened by forming the gate electrode on the overhang portion of the lamination film 10c. Therefore, the control voltage to be applied to the gate electrode can be lowered and the performance of the field emission element can be improved. 30

The present invention has been described in connection with the preferred embodiments. The invention is not limited only to the above embodiments. It is apparent that various modifications, improvements, combinations, and the like can be made by those skilled in the art.

I claim:

1. A method for fabricating a field emission apparatus, comprising the steps of:
  - a) providing a substrate having a mask layer thereon;
  - b) selectively removing the mask layer to provide a window;
  - c) isotropically removing the substrate through the window to provide a hollow space in the substrate, wherein the hollow space laterally spreads through the window to the underneath of the mask layer;
  - d) providing a sacrificial layer over the window and the mask layer so as to provide sacrificial films laterally separated along a horizontal direction of the substrate;
  - e) at least partially reacting the sacrificial films in such a manner that the reacted sacrificial films are brought into contact with therewith after the completion of the reaction so as to provide a cusp mold on the reacted sacrificial films; and
  - f) providing an electron emitting layer over the reacted sacrificial films.
2. A method according to claim 1, wherein the mask layer is made of a material selected from a group consisting of  $\text{SiN}_x$ ,  $\text{SiO}_2$ ,  $\text{AlN}_x$ , and  $\text{Al}_2\text{O}_3$ . 60
3. A method according to claim 1, wherein the substrate is made of a material selected from a group consisting of Si and Al. 65
4. A method according to claim 1, wherein the sacrificial layer is made of polysilicon.

## 12

5. A method according to claim 1, wherein the step d) is performed by wet oxidation.

6. A method according to claim 1, wherein the electron emitting layer is made of TiN.

7. A method according to claim 1, further comprising the step of:

d-1) implanting ions into the sacrificial films, following the step d).

8. A method according to claim 5, wherein the reacted sacrificial films are made of  $\text{SiO}_2$ .

9. A method for fabricating a field emission apparatus, comprising the steps of:

a) providing a substrate having a mask layer thereon;

b) selectively removing the mask layer to provide a window;

c) isotropically removing the substrate through the window to provide a hollow space in the substrate, wherein the hollow space laterally spreads through the window to the underneath of the mask layer;

d) providing a first sacrificial layer over the window and the mask layer so as to provide sacrificial films laterally separated along a horizontal direction of the substrate;

e) providing a second sacrificial layer on the sacrificial films;

f) at least partially reacting the sacrificial films with the second sacrificial layer to provide a cusp mold on the reacted sacrificial films; and

g) providing an electron emitting layer over the reacted sacrificial films.

10. A method according to claim 9, wherein the first sacrificial layer is made of a material selected from a group consisting of polysilicon and amorphous silicon.

11. A method according to claim 9, wherein the second sacrificial layer is made of a material selected from a group consisting of Ti, Ta, Mo, and W.

12. A method according to claim 9, further comprising the step of:

f-1) removing an unreacted portion of the second sacrificial layer, following the step f).

13. A method for fabricating a field emission apparatus, comprising the steps of:

a) providing a substrate having a mask layer thereon;

b) selectively removing the mask layer to provide a window;

c) isotropically removing the substrate through the window to provide a hollow space in the substrate, wherein the hollow space laterally spreads through the window to the underneath of the mask layer;

d) providing a sacrificial layer over the window and the mask layer so as to provide sacrificial films laterally separated along a horizontal direction of the substrate;

e) reacting the sacrificial films in such a manner that the reacted sacrificial films are brought into contact therewith after the completion of the reaction so as to provide a cusp mold on the reacted sacrificial films while an unreacted portion of the sacrificial layer is remained under the reacted sacrificial films;

f) providing an electron emitting layer over the reacted sacrificial films;

g) forming holes in the electron emitting layer; and

h) selectively removing the reacted sacrificial films through the holes in the electron emitting layer, wherein the unreacted portion of the sacrificial layer is served as a gate electrode.

**13**

**14.** A method according to claim **13**, wherein the sacrificial layer is made of polysilicon.

**15.** A method according to claim **13**, wherein the electron emitting layer is made of TiN.

**14**

**16.** A method according to claim **13**, wherein the step h) is performed by wet etching.

\* \* \* \* \*